

No. 622,800.

Patented Apr. 11, 1899.

G. M. HATHAWAY.  
DETONATING COMPOUND.

(Application filed Feb. 14, 1898. Renewed Sept. 16, 1898.)

(No Model.)

Fig. 1



Fig. 3.

WITNESSES:

I. W. Johnson,  
H. H. Norton

INVENTOR  
Geo. M. Hathaway  
BY  
A. P. Nottingham  
ATTORNEY.

# UNITED STATES PATENT OFFICE.

GEORGE M. HATHAWAY, OF NEW YORK, N. Y., ASSIGNOR TO M. C. ARNOT,  
OF ELMIRA, NEW YORK.

## DETONATING COMPOUND.

SPECIFICATION forming part of Letters Patent No. 622,800, dated April 11, 1899.

Application filed February 14, 1896. Renewed September 16, 1898. Serial No. 691,086. (No specimens.)

*To all whom it may concern:*

Be it known that I, GEORGE M. HATHAWAY, a citizen of the United States, residing at New York, in the county of New York and State 5 of New York, have invented certain new and useful Improvements in Detonating Compositions; and I do hereby declare the following to be a full, clear, and exact description of the invention, such as will enable others skilled 10 in the art to which it appertains to make and use the same.

The invention relates to certain improvements in detonating compounds for exploding high explosives of any description, but is especially designed to explode the compound or compounds known in the market as "joveite," which consists, essentially, in the combination of a suitable hydrocarbon derivative, an oxidizing agent, and a suitable material for 15 rendering the compound sufficiently sensitive to be detonated or exploded, such as a composition of nitro-naphthalene, nitro-phenol, and nitrate of soda, or nitro-naphthalene, nitro-phenol, and nitrate ammonia.

20 The principal object of the invention is to furnish a thoroughly safe and reliable detonator by means of which the explosive known as "joveite" can be successfully exploded when in a solidified or tightly-packed form 25 and which cannot be exploded by any means other than by fire or flame.

Experience has demonstrated that a more powerful explosion takes place when the joveite is in a compressed or solidified form than 30 when in a granulated condition; but the great difficulty has been to obtain a composition that would successfully detonate or explode the compound when in this form. The percussive force of the ordinary fulminates will 35 not accomplish it, as their action is entirely too quick. After many experiments I have found that a detonating composition of low 40 grade, which explodes less suddenly and is virtually devoid of percussive force, must be employed.

45 While the invention is designed to furnish a detonator for exploding shells and other projectiles charged with the high explosive compound for military and naval purposes, 50 it is equally well adapted for use in blasting purposes, wherein the explosive is molded into

sticks and inserted in holes made in rocks and in which the ordinary detonator fails to act reliably.

My composition is composed of the following-named ingredients, which are designated by the letters A, B, C, D, E, F, and G, grouped and inclosed by brackets as herein below:

|                             |    |    |
|-----------------------------|----|----|
| (A) Charcoal .....          | 15 | 60 |
| (B) Sulfur.....             | 10 |    |
| (C) Saltpeter.....          | 75 |    |
| (D) Nitro-naphthalene ..... | 5  |    |
| (E) Nitro-phenol .....      | 35 | 12 |
| (F) Nitrate of soda .....   | 5  |    |
| (G) Chlorate of potash..... | 3  | 65 |

The ingredients charcoal, sulfur, and saltpeter are pulverized and thoroughly mixed, and the ingredients nitro-naphthalene, nitro-phenol, and nitrate of soda are mixed at a 70 temperature of about 200° Fahrenheit and ground together while in this heated condition. After being thus thoroughly mixed the compound of charcoal, sulfur, and saltpeter forms one part of my composition and 75 nitro-naphthalene, nitro-phenol, and nitrate of soda constitute the second part thereof, and for the purpose of facilitating the future description of the composition I will herein-after refer to those parts as 1 and 2. The 80 parts 1 and 2 are then added together in the proportions indicated above and are thoroughly mixed while in a heated condition, so as to remove all moisture. After the parts 1 and 2 have been thoroughly mixed and dried 85 the ingredient chlorate of potash, which constitutes the third part and which is in the form of an impalpable powder, is then distributed or sprinkled over said parts 1 and 2 and carefully mixed therewith, the distributing or 90 sprinkling being continued at intervals until the composition has received the full amount of the chlorate of potash. The mixture thus formed is then heated to about 90° Fahrenheit, so as to thoroughly dry and remove all 95 moisture. It is then ground, mixed with water in sufficient quantity to form a stiff pasty mass, and caked and granulated to form the detonating composition.

The nitrate of potash or ammonia furnishes 100 one of the oxidizing agents of the compound; but such does not give off its oxygen with suf-

ficient rapidity to cause the composition when fired to detonate the joveite. The chlorate of potash constitutes another oxidizing agent. This parts with its oxygen freely and rapidly, 5 and if used alone as the oxidizing agent would form a percussive compound wholly unfitted for a detonator. The nitrates above mentioned act to modify the explosive force so as to produce a detonator which, having virtually no percussive force, is more rapid in its action than the composition in which nitrates alone are employed as the oxygen-furnishing agents.

The discharge of all detonators causes more or less vibratory motion of all substances adjacent thereto; but the compositions containing the nitrates alone as the oxidizing agent give rise to vibrations which are too slow to break up the mass of joveite when compacted 20 and at the same time communicate the fire from the detonator thereto, while the chlorate when employed alone as an oxidizing agent causes too rapid vibrations or percussive action, which ruptures the packed mass of explosive and scatters it before the flame can take effect. By the use of the two oxidizing agents—that is, a nitrate and a chlorate—a vibratory action will be set up which will disrupt the surrounding mass and permit the fire 25 to be simultaneously communicated thereto.

The phenol derivatives and the nitro-naphthaline derivatives employed are the nitro derivatives consisting of mixtures of substances having various degrees of nitration. In the 30 nitro derivatives of phenol (the nitro used in this process) there is generically contained from ten per cent. to twenty-five per cent. of tri-nitro-phenol, the remaining constituent being a mixture of mono and di-nitro phenol.

In the accompanying drawings are shown two means of employing my new composition, Figure 1 representing a sectional view of a detonator and time-fuse plug to be used in exploding a shell or other projectile, Fig. 2 a 40 sectional view showing the parts in position and properly shaped, and Fig. 3 a sectional view showing a detonator charged and provided with a tape-fuse and applied to a stick of joveite.

The detonator shown in Figs. 1 and 2 consists of a shouldered plug 1, having an extended tube 2, which extends into the shell (not shown) when the detonator is in place,

the plug back of the shoulder being externally screw-threaded, so as to fit the internal 55 threads of the opening in said shell or projectile. The plug is bored from its rear to the front, and the bore is screw-threaded to receive an externally-screw-threaded time-fuse plug 3, which is provided with a longitudinal bore of small diameter. The said bore is charged with fuse-powder, and at its rear end is seated a percussion-cap provided with the usual anvil, by means of which cap the fuse-powder may be fired on the impact 60 of the shell by a striker, which is arranged in the fuse-case of the shell.

As shown in Fig. 3, the detonator is represented as embedded in one end of a stick of joveite. In this instance the detonator consists of a metallic tube 5, closed at one end and open at the other. The said tube is filled with the detonating composition and is externally screw-threaded at one end to be received into one end of a fuse-tube 6, which 70 holds a tape-fuse 7. The tube 6 is crimped at intervals to hold the tape-fuse against displacement, as shown in said Fig. 3.

The detonating compound is ignited by means of a fuse, which may be either a time-fuse, a fuse to be fired by a percussion-cap, or a tape-fuse. In either case the fire is communicated from said fuse to the detonating compound and from the said compound to the surrounding mass of joveite, a terrific explosion 80 being the result.

Having thus fully described my invention, what I claim, and desire to secure by Letters Patent, is—

1. A detonating compound, composed of 90 the ingredients of gunpowder, with nitro-naphthalene, nitro-phenol, nitrate of soda, and chlorate of potash, combined in such proportions as to form a detonating compound of low grade.
2. A detonating compound, composed of charcoal, sulfur, saltpeter, nitro-naphthalene, nitro-phenol, nitrate of soda and chlorate of potash, in about the proportions specified.

In testimony whereof I affix my signature in the presence of two witnesses.

GEORGE M. HATHAWAY.

Witnesses:

J. R. NOTTINGHAM,  
L. L. JOHNSON.